

## [54] PRODUCTION OF TEXTURISED YARN

[75] Inventors: Werner Doschko, NuBloch, Am Leimbach; Hermann Rinklin, Oestringen, both of Germany

[73] Assignee: Imperial Chemical Industries Limited, London, England

[22] Filed: Nov. 6, 1972

[21] Appl. No.: 304,033

## [30] Foreign Application Priority Data

Nov. 17, 1971 Great Britain ..... 53300/71  
July 13, 1972 Great Britain ..... 32813/72

[52] U.S. Cl. ..... 57/34 HS, 57/51.6, 57/157 TS,  
57/157 MS, 57/56

[51] Int. Cl. ..... D02g 1/02  
[58] Field of Search ..... 57/1 R, 34 R, 34 HS, 36,  
57/51, 51.6, 157 R, 157 S, 157 MS, 157 TS,  
56

## [56] References Cited

## UNITED STATES PATENTS

2,936,567 3/1960 Russell et al. ..... 57/77.4

|           |         |                     |             |
|-----------|---------|---------------------|-------------|
| 3,041,814 | 7/1962  | Held .....          | 57/34 HS    |
| 3,069,837 | 12/1962 | Olson .....         | 57/34 HS X  |
| 3,178,795 | 4/1965  | Warthen .....       | 57/34 HS X  |
| 3,365,874 | 1/1968  | Chidgey et al. .... | 57/157 TS   |
| 3,432,355 | 12/1947 | Truitt .....        | 57/157 S X  |
| 3,645,081 | 2/1972  | Salama .....        | 57/34 HS    |
| 3,651,633 | 3/1972  | Steinmiller .....   | 57/157 TS X |
| 3,729,916 | 5/1973  | Lusk et al. ....    | 57/34 HS    |

Primary Examiner—Donald E. Watkins  
Attorney, Agent, or Firm—Herbert M. Adrian, Jr.

[57]

## ABSTRACT

A process for producing bulk is described by sequentially drawing and false twist texturizing a synthetic yarn wherein the yarn is withdrawn from the texturizing zone at a greater speed than it is fed thereto. In a preferred embodiment, the draw roll for the drawing step also serves as the take-off roll for the texturizing zone and is stepped so that the portion used to take off the texturized yarn is of greater diameter than the part used for drawing. A further preference is that the heater in the texturizing zone is a heated pin.

15 Claims, 2 Drawing Figures



PATENTED AUG 13 1974

3,828,537

SHEET 1 OF 2



PATENTED AUG 13 1974

3,828,537

SHEET 2 OF 2



## PRODUCTION OF TEXTURISED YARN

The present invention relates to improvements in or relating to the production of texturised yarn. In particular the present invention is concerned with the production of texturised yarn by the false twist principle. False twisting is a technique which is used to produce a texturised effect in yarns and a false twist is conveniently achieved by first passing a moving yarn through a region where it is heated to above the second order transition temperature of the materials from which the yarn is made then allowing the yarn to cool and twisting the cooled yarn. The twist imparted to the cooled yarn runs back along the yarn in the opposite direction to that in which it is travelling and into the heating zone so that the twist is set in the yarn when it moves into the cooling zone and the temperature drops below the second order transition temperature.

After the yarn has passed through the twisting device, it is allowed to untwist so that the untwisting of the yarn which has been set in its twisted state results in a texturised or bulked yarn.

Many fabrics require a high level of bulk in the yarn particularly stretch fabrics as are used in ladies stockings. The bulk in fabric made from texturised yarn is mainly dependent on the twist density of the yarn in the heating zone. By twist density we mean the number of twists per unit length in the yarn. Twist density is controlled by the nature and physical properties of the yarn supplied, ie, its chemical type, titre, number of filaments in the cross section and by the physical properties of the filaments, and also by the imposed processing conditions, namely yarn speed, twist speed, time and temperature of heating and cooling, frictional forces in the twisting device and the nature and amount of lubricant on the surface of the yarn. It has been difficult to produce texturised yarn capable of developing a constant high level of bulk whilst having a low thermal shrinkage and an aim of our invention is to provide such a yarn and a convenient method for its production.

One problem that arises while texturising on a commercial scale is that the processing conditions tend to vary from one position on a machine to another. This tends to result in non-uniform yarn which shows up as stripes in fabrics produced from the yarn for example the rings which sometimes appear in ladies stockings. It is thought that this non-uniformity is at least partly due to inadequate contact between the yarn and both the heater and twist bush in the texturising zone which results in variations in the amount of twist inserted and the degree to which the twist is set. It is an object of the present invention to improve this uniformity.

Various devices are known for imparting twist to a moving yarn. In one such device the moving yarn is passed around a member which is provided within and rotates with a hollow spindle. In this way twist is inserted in the yarn as it passes through the spindle. This technique is limited in the amount of twist that can be inserted in a yarn travelling at a particular speed as it is only possible to insert one twist for every rotation of the spindle. Alternative techniques for imparting twist which overcome this limitation use the friction principle whereby the yarn is twisted by contact with a rotating friction surface. The twist devices which use the friction principle generally consist of rotating hollow surfaces with which the moving yarn makes contact. In

some such devices the yarn passes through the cylindrical body whereas in others the yarn enters and leaves the body from the same side and is held against the friction surface by a yarn guide.

The present invention is concerned with the production of texturised yarn by the friction false twist principle because this allows a greater degree of twist to be inserted into the yarn for a given speed of rotation of the twist bush and thus allows higher processing speeds to be used. It has already been proposed to produce texturised yarn by sequentially stretching and texturising by using the same roll to withdraw the yarn from both the texturising and the stretching zones. However, in this earlier process the roll that is used is stepped and the yarn passes around the portion of smaller diameter after passing through the texturising zone so that the yarn tension is relaxed while it is passing through the texturising unit compared to its state in the stretching zone. We have found that this process results in yarn having a non-uniform and comparatively low level of bulk. It has also been proposed that yarn may be partially drawn and then simultaneously texturised and drawn to complete drawing. This process however suffers from the disadvantage that the yarn speed and the tension in the yarn during texturising are fixed according to the required draw ratio and thus the process allows no freedom to control the yarn speed during texturising to ensure that the necessary degree of bulk is achieved. Furthermore, this process requires a comparatively high stretch in the texturising zone which tends to remove some of the twist during heating resulting in yarn having an undesirably low level of bulk. We have now found that providing certain conditions are used yarn having a desired high level of bulk as shown by its crimp rigidity may be obtained.

The present invention therefore provides a process for the production of texturised yarn wherein thermoplastic synthetic yarn is sequentially stretched and texturised by the friction false twist principle as hereinbefore described wherein the yarn is fed continuously from the stretching zone to the texturising zone and the yarn leaves the texturising zone at a greater speed than that at which it enters the said texturising zone.

It is to be understood that the present invention is concerned only with a process where the increase in speed in the texturising zone is comparatively small and is not of the same order as speed increases generally used for stretching yarn. Whilst the actual speed increase used depends upon the particular yarn we generally find that it should be no greater than a 10% increase.

The process of the present invention may be applied to the production of yarn from any thermoplastic synthetic material which when twisted at a temperature above its second order transition temperature and then cooled whilst in its twisted state becomes set in that twisted state. Examples of particularly useful thermoplastic synthetic materials include Nylon 6, Nylon 6,6, polyacrylonitrile and thermoplastic polyesters such as polyethylene terephthalate.

In our preferred process the unstretched yarn first passes from a feed station to a draw roll so that the yarn is stretched between the feed station and the draw roll. The yarn is then fed directly from the draw roll through a heater zone which we prefer be a pin heater around which the yarn is wrapped as this ensures quick heating and uniform heat transfer between the yarn and the

heater and allows higher speed processes to be used. It is thought that the techniques of the present invention are particularly suited to processes using a pin heater because the slight increase in yarn speed in the texturising zone ensures good contact between the yarn and the pin heater to give consistent heating in addition to good contact between the yarn and the friction bush to give a more constant level of twist. A further advantage of using a pin heater is that the extent to which the yarn is heated may readily be altered by varying the wrap of the yarn around the heater. In addition a pin heater has the added advantage that it occupies considerably less space for the same degree of heating than the plate heaters traditionally used in processes of this type. If the increase in speed in the texturising zone is too great some of the bulk inserted by the bush will be pulled out by the high tension. If, however, there is a reduction in yarn speed during texturising the yarn will not be held sufficiently firmly against the friction bush to impart adequate twist to the yarn nor against the heater to ensure adequate setting of the twisted yarn. After the yarn has passed the heater it is cooled to ensure that it is cold when it reaches the twist device, and it may be necessary to provide cooling plates which direct cold air on to the yarn, but generally we find it more convenient to ensure that the distance the yarn travels between the heater and the twist device is sufficient to cool the yarn.

After cooling the yarn passes to the twisting device which may be any of the known friction devices for imparting twist to yarns, in particular twist bushes. The twist imparted to the yarn runs back along the yarn to the heater so that the yarn is twisted when hot and the hot twisted yarn then cools thus setting the yarn in its twisted state. According to the friction false twist technique the twist device provides a rotating friction surface with which the yarn is brought into contact so that the rotation of the friction surface imparts a twist to the yarn. The yarn is withdrawn from the twist device in such a way that the speed of withdrawal is greater than the speed of the yarn as it is fed to the twist device. In a preferred embodiment the yarn is withdrawn from the twist device by the roll that is used as the draw roll of the stretching zone. In this particular technique, the roll is stepped so that the portion around which the yarn passes at the end of the draw zone is of smaller diameter than the portion around which the yarn passes after the texturising zone so that the speed of the yarn is increased between the two portions of the roll. This technique is preferred as the dual functions of a single roll results in a more compact apparatus.

The preferred amount by which the yarn speed should be increased in the texturising zone depends upon the nature, denier and amount of twist to be inserted into the yarn. However, we have found that for certain yarns there are limits for the speed increase within which the desired high crimp rigidity is obtained. We find that these limits are generally within the elastic limit of the yarn and thus our process usually results in no permanent stretch of the yarn as it passes through the texturising zone over and above any stretch imparted by the texturising action. This is apparent by a comparison of the average decitex of the yarn produced by our preferred process with the average decitex of yarn produced by a similar process without any speed increase in the texturising zone which shows virtually no difference in the decitex of the two yarns.

However, in some instances the increase in speed may be such as to result in a slight permanent stretch but this is generally very small. The preferred increase in yarn speed depends upon the particular type of yarn. 5 However, we have found that a speed increase between 2 and 10% is to be preferred. In particular, we find that an increase in yarn speed of between 2 and 6% is suitable for the production of texturised polyamide yarn. A speed increase of this magnitude during texturising 10 produces virtually no more permanent stretch than a similar process with no such speed increase.

After the yarn has been withdrawn from the texturising unit, it is fed to the wind-up. We have found that the process of the present invention enables a yarn of high 15 crimp rigidity to be obtained which is particularly important for yarns to be used in fabrics where fabric bulk and high elasticity are required such as for example in ladies stockings. In addition the yarns produced by our process have a sufficiently low shrinkage that a fabric 20 made from the yarn does not alter appreciably during fabric finishing. We have also found that the slight speed increase in the texturising zone results in improvements in both the uniformity of the yarn obtained from one position on a machine and between the yarns 25 obtained from different positions. This is thought to arise from greater yarn stability and in some instances it is possible to see that the threadline is more stable during texturising than in similar processes with no speed increase during texturising. This improved stability 30 also leads to a smoother running process shown by the fact that threadline breaks occur less frequently when using the process of the present invention.

The crimp rigidity of a yarn is a measure of the ability 35 of a texturised yarn to develop bulk during finishing and of the ability of the yarn to retain the bulk. The higher the crimp rigidity the greater the degree of bulk and the more elastic the yarn. For the purposes of this specification crimp rigidity is determined by making a 40 loop from the texturised yarn and initially hanging a weight of 0.1 grams per decitex on the yarn and suspending the weighted skein in water at 20°C for 2 minutes. The length of the skein is then measured. The weight is then replaced by a weight of 0.002 grams per decitex and the length of the skein measured under 45 similar conditions. The crimp rigidity is the ratio of the length under a load of 0.002 grams per decitex to the length under a load of 0.1 grams per decitex expressed as a percentage. In particular, by using the process of 50 our invention we have obtained yarn having a crimp rigidity of from 35% to 50% and a shrinkage of less than 5%; the crimp rigidity that may be achieved is of course dependent on the decitex of the yarn.

In a preferred embodiment of the present invention 55 a twist damming element is positioned in the yarn path between the draw roll and the heater. The term twist damming element refers to any system which prevents twist running along a yarn and may be a pin around which the yarn is wound although this is not preferred as such a dramatic change in yarn direction can cause filamentation and damage to the yarn. We do therefore prefer to use a system in which the direction of the yarn path is changed as gradually as possible consistent with achieving the necessary degree of twist damming. We have found that a particularly useful twist damming element 60 comprises a series of yarn guides which are preferably rolls or ceramic guides around which the yarn passes wherein the yarn path is forced to change by at 65

least 75° as it passes around each roll. We find the inclusion of a twist damming element useful as it prevents the twist inserted by the twist device from running back onto the draw roll. If the yarn is twisted on the draw roll an inferior product can result as tension fluctuations in the draw zone can occur giving rise to non-uniform drawing and a variable product. Furthermore, the yarn tends to roll on the surface of the roll so that adjacent strands become intertwined, thus stopping operations. In addition if the yarn moves on the surface of a roll which controls yarn speed due to the torque imparted by texturisation the surface of the roll becomes quickly damaged. The use of a twist damming element has an added advantage when used in conjunction with a pin heater as if the damming element is a movable yarn guide its position may readily be altered to provide any easy method of varying the wrap of the yarn around the pin heater.

The essence of our invention is therefore a continuous stretching and texturising process in which the yarn speed is increased during texturising. It should be understood that this principle may be applied to a process in which the yarn is first simultaneously stretched and texturised and then subsequently further texturised. In this embodiment the speed of the yarn will be increased during the further texturising. Similarly the texturised yarn produced by our process may be further texturised if required. Both these processes are aimed at ensuring even greater uniformity of the final bulked yarn.

The yarn produced by the process of this invention is a torque yarn as it has been twisted in one direction about its axis. However, if a torque free yarn is required, our process may be applied to two separate yarns which pass through the apparatus in parallel and are subjected to equal amounts of twist but in the opposite direction. The yarns may then be combined to form a torque free composite yarn.

The present invention also provides an apparatus for sequentially stretching and texturising yarn comprising a draw zone with feed means and a drawing means and a texturising zone comprising a feed roll, a heater, a friction texturising device and a withdrawing means wherein the feed roll also acts as the withdrawing means for the texturising zone and is stepped so that it is the portion of larger diameter that acts as the withdrawing means.

The various modifications and embodiments of the apparatus of the present invention corresponds to the embodiments of the process already described.

The present invention is illustrated but in no way limited by reference to the accompanying diagrammatic drawing FIG. 1. Undrawn yarn 1 is delivered to feed roll 2 from which it passes to the draw pin 3 and then to draw roll 5. The draw roll 5 is stepped and the yarn

justed so that the yarn is stretched to the desired extent. After passage around the portion 6, the yarn passes to heated pin 7 where it is heated to a temperature above the second order transition temperature of the material from which the yarn is made. The yarn then passes to yarn guide 8 and into the friction twist bush 9. The yarn path between the heated pin 7 and the pin guide 8 is sufficiently long to ensure that the yarn is no longer "tacky" when it passes through the guide 8.

In the type of twist bush illustrated, the yarn passes through the bush and it is twisted by frictional contact between the inner surface of the bush and the yarn. The twist imparted to the yarn runs back along the yarn towards the heated roll 7 so that the yarn is twisted while hot and the twist is set in the yarn as it cools. The yarn passes from the twist bush through another yarn guide 10 to the larger diameter portion 11 of the roll 5. From the portion 11, the yarn travels around the separator roll 4, back to the portion 11 of roll 5, back to the separator roll again, through the yarn guide 8 and is wound up on the bobbin 12 by means of the ring and traveller 13. Thus, the speed of the yarn is increased as it passes through the texturising zone because it is fed to the zone at the peripheral speed of the smaller portion of roll 5 and is withdrawn at the peripheral speed of the larger portion.

The present invention is further illustrated but in no way limited by reference to the following examples throughout which any reference to the decitex of the yarn refers to the decitex after texturising.

#### EXAMPLE I

35 Twenty-two decitex 7 filament Nylon 66 yarn was processed using the apparatus illustrated in FIG. 1. The draw roll 5 was driven so that the portion of smaller diameter 6 was rotating at a peripheral speed of 685 metres per minute to draw the yarn to a ratio of 2.66. The 40 twist bush 9 was rotated at a speed of about 21,500 revolutions per minute and the heated pin 7 was maintained at a temperature between 220° and 230°C. the roll 5 was stepped so that the peripheral speed of the larger portion 11 was 4% greater than that of the 45 smaller diameter portion 6.

For the sake of comparison, an identical sample of yarn was processed in exactly the same manner with the exception that after passage through the texturising zone, the yarn did not pass over the larger diameter 50 portion of roll 5 (i.e. portion 11) but passed once again over the portion 6 so that the yarn was not subject to any increase in speed during texturising.

The properties of the two yarns obtained are set out in the following table:

|                    | With 4% increase in yarn speed in texturising zone | With no speed increase |
|--------------------|----------------------------------------------------|------------------------|
| Crimp Rigidity     | 51%                                                | 41%                    |
| Extension to Break | 28.7%                                              | 28.0%                  |
| Breaking Load      | 96 grams                                           | 96 grams               |
| Tenacity           | 4.42 grams/decitex                                 | 4.42 grams/decitex     |
| Titer of Yarn      | 21.7                                               | 21.8                   |
| Hot Shrinkage      | 4.5%                                               | 5.5%                   |

from the draw pin 3 passes to the portion 6 which has the smaller diameter. The yarn then travels to the separator roll 4 and again to the portion 6. The relative speeds of the feed roll 2 and the draw roll 5 are ad-

Thus it may be seen that by employing the process of the present invention, yarn having an improved crimp rigidity and a lower shrinkage may be obtained without impairing other yarn properties. The yarn was subse-

quently knitted into stockings which after dying and finishing had excellent appearance and uniformity.

The hot shrinkage of the yarn is determined by taking a 1 metre length of yarn that has been stored for at least 24 hours under normal conditions. The length of yarn is made into a single loop and subjected to a tension of 18 grams/decitex and the length of the loop measured ( $L_1$ ). The loop of yarn is then suspended in boiling water for 15 minutes, dried under normal conditions for 24 hours, re-subjected to a tension of 18 grams/decitex and the length of the loop measured ( $L_2$ ).

The percentage shrinkage is given by  $(L_1 - L_2)/L_1 \times 100$ .

The crimp rigidity of the yarn is measured by the technique previously described.

#### EXAMPLE II

The process of Example I was repeated but using a 44 decitex 14 filament polyamide yarn and a twist bush speed of 12,500 revolutions per minute. Several runs were carried out in which the speed at which the yarn was withdrawn from the texturising zone compared to the speed at which it was drawn off from the draw zone was varied from 6% below that at which it was withdrawn from the draw zone to 10% above that at which it was withdrawn from the draw zone. The crimp rigidity of each sample was measured by the method described above and FIG. 2 is a plot of crimp rigidity against the amount by which the yarn speed is increased through the texturising zone. As may be seen the curve passes through a peak at about 4% increase in speed.

#### EXAMPLE III

The process of Example I was repeated using a 3 filament 17 decitex polyamide yarn. The draw roll 5 was driven so that the portion of smaller diameter was ro-

Accordingly it may be seen that in all instances the process of the present invention produced yarn of improved crimp rigidity. In addition these results show that the speed increase results in a higher yarn tension before the heater which gives rise to improved running.

#### EXAMPLE IV

The process of Example I was repeated using a 3 filament 17 decitex polyamide yarn. The portion of the draw roll which withdraws the yarn from the draw zone was rotating at a peripheral speed of 674 metres per minute and the roll was stepped to give an 8% increase in speed between the beginning and the end of the texturising zone. The temperature of the heated pin was about 230°C and the yarn thread up was such that the yarn passed once around the pin. The yarn obtained contained 7,100 twists per metre, had a crimp rigidity of 41.5% and a shrinkage of 5.3%. Tension measurements on the yarn during processing showed that the tension before the heater was 2.4 grams, immediately after the heater it was 6.8 grams and after the twist bush 12.5 grams.

As may be seen in Examples III and IV the increase in the speed of the yarn in the texturising zone results in an increase in yarn tension compared to a similar process with no speed increase during texturising. It is this increase in tension which is thought to result in more uniform running and few yarn breaks because yarn has a tendency to stick to the processing rolls which can result in fluctuations of the conditions to which the yarn is subjected and this tendency is reduced by the higher tensions we produce. Our invention therefore provides a simple method of overcoming this disadvantage. Tension measurements were also made during the production of 14 filament 44 decitex polyamide yarn passing round a 4 inch diameter pin heater held at a temperature of 230°C; the results were as follows:

| Speed Change of Yarn<br>in Texturising Zone | Tension in Yarn (grams) |                                  |                     |
|---------------------------------------------|-------------------------|----------------------------------|---------------------|
|                                             | Before heater           | Between heater<br>and twist bush | After twist<br>bush |
| Speed Decreased by 4%                       | 2                       | 10.5                             | 18.5                |
| No Change                                   | 3.5                     | 13.5                             | 24.0                |
| Speed Increased by 4%                       | 4.8                     | 16.5                             | 29.5                |

tating at a peripheral speed of 650 metres per minute to draw the yarn to a draw ratio of 2.99. The heated pin was maintained at a temperature in the range 185° - 195°C and the roll 5 was stepped to give the same 4% increase in yarn speed as in Example I.

Three experiments were carried out using different speeds of rotation of the twist bush and each run was compared with a similar process with no increase in yarn speed in the texturising zone. The comparative results were as follows:

| Bush Speed<br>r.p.m. | Crimp Rigidity (%)           |                                 | Shrinkage (%)                |                                 | Yarn Tension (grams)         |                                 |
|----------------------|------------------------------|---------------------------------|------------------------------|---------------------------------|------------------------------|---------------------------------|
|                      | With 4%<br>speed<br>increase | Without<br>4% speed<br>increase | With 4%<br>speed<br>increase | Without<br>4% speed<br>increase | With 4%<br>speed<br>increase | Without<br>4% speed<br>increase |
| 17,400               | 38.5                         | 32.5                            | 7.8                          | 7.4                             | 2.6                          | 2.3                             |
| 20,100               | 40.5                         | 34.3                            | 7.1                          | 7.2                             | 3.0                          | 2.5                             |
| 22,800               | 42                           | 38.5                            | 5.6                          | 5.8                             | 3.2                          | 2.8                             |

The yarn produced by the process involving a 4% increase in speed produced more uniform fabrics and also ran much more smoothly during texturising than the other yarns.

The increase in tension before the heater is important when a pin heater is used as the wrap of the yarn around the pin heater reduces the yarn tension before the heater and there is a risk that the tension will become so low that the yarn will occasionally stick to the roll that feeds it to the texturising zone. Our invention

provides a comparatively simple method of overcoming this problem.

We claim:

1. A process for false twist texturing a synthetic filament yarn comprising sequentially passing the yarn being treated through a drawing zone, a twist heat setting zone, a twisting zone, an untwisting zone and a yarn speed increase zone prior to take up wherein the yarn is first drawn to the desired extent prior to passing to the twist heat setting zone and twisting zone, said yarn being twisted and the twist being passed upstream into the twist heat setting zone wherein said yarn is heated to above its second order transition temperature to set said yarn in the twisted configuration, untwisting said heat set yarn, increasing the speed of said yarn up to about 10 percent as it passes through said heat setting and twisting zone and subsequently taking up a textured yarn.

2. The process of claim 1 wherein the yarn is a polyester continuous filament yarn.

3. The process of claim 1 wherein the yarn is a polyamide continuous filament yarn.

4. The process of claim 1 wherein the yarn speed increases as it passes through said heat setting and twisting zone by 2 to 10 percent.

5. A process according to claim 4 in which the yarn speed increases by between 2 and 6%.

6. A process according to claim 1 in which the increase in speed in the yarn as it passes through the heat setting and twisting zone is such that it produces no permanent stretch in the yarn.

7. The process of claim 1 wherein the yarn passes through a twist damming zone prior to passing through

said twist heat setting zone.

8. The process of claim 7 wherein the twist damming zone comprises passing the yarn through a path of curvature equalling at least a 75° turn.

9. A process according to claim 1 in which the yarn is also texturised in the stretching zone.

10. A process according to claim 1 in which the textured yarn is further texturised.

11. An apparatus for sequentially stretching and texturising yarn comprising a draw zone with means for feeding the yarn to a texturising zone and drawing means to withdraw the yarn from said texturising zone and to effect the required drawing of the yarn and said texturising zone comprising a feed roll, a heater, a friction texturising device providing a friction surface which bears against the yarn and a means for withdrawing the yarn wherein the feed roll also acts as the withdrawing means and is stepped so that it is the portion of larger diameter which acts as the withdrawing means.

12. An apparatus according to claim 11 in which the heater in the texturising zone is a heated pin with which the yarn makes contact.

13. An apparatus according to claim 11 in which the feed roll for the texturising zone is also the drawing means for the draw zone.

14. An apparatus according to claim 11 in which the diameter of the portion of the feed roll is between 2% and 10% larger than the other portion of the roller.

15. An apparatus according to claim 11 including a twist damming element with which the yarn makes contact between the heated pin and the draw roll.

\* \* \* \* \*

35

40

45

50

55

60

65